

Patented June 4, 1929.

1,716,120

# UNITED STATES PATENT OFFICE.

CHARLES S. FRIEDMAN, OF PARIS, FRANCE, ASSIGNOR TO SOCIÉTÉ: ANCIENS ETABLISSEMENTS A. COMBE & FILS & CIE., OF PARIS, FRANCE.

## PROCESS FOR THE PRODUCTION OF WASHABLE PRINTINGS ON LEATHER.

No Drawing. Application filed April 13, 1923, Serial No. 631,954, and in France November 30, 1922.

Heretofore, the only hides or skins used for the production of printings were those which have been tanned with vegetal substances, like those which are used for making morocco-leather goods, for furniture, book-bindings, fancy articles, millinery and dress-making. Besides this, the leather and the printing would not resist washing.

The present invention relates to a process 10 for producing washable printings upon leather, with the purpose of obtaining articles, which besides being adapted for the above mentioned purposes, may compete with the polychromatic fabrics as used actually 15 for shoes, slippers and the like, which they imitate in appearance and of which they possess the softness.

According to the invention, the hide or skin is first tanned with formol in the usual 20 manner, this tanning operation enabling the hide or skin to subsequently withstand, after printing, a temperature sufficiently high to fix the dye-stuffs used for printing fabrics.

After the operation of tanning with formol, the hides or skins are submitted to a new 25 tanning operation in a bath of powdered sumach or any other similar substance, for an hour, at a temperature of 35° C.

They are for instance mechanically treated 30 in the usual manner in order to give them the appearance of velvet, or suede leather; in other words, the hides or skins receive an ooze or suede, or any other, finish.

After having been dried at 35° C., the hides 35 or skins are then ready to be printed. This operation is performed by means of engraved plates, with the employment, for example, of the following mixture:

40 25 to 30 grams of dye-stuff (Rhodamine).  
200 to 500 grams of tragacanth.  
40 to 60 grams of acetate of chrome.  
5 to 10 grams of tannic acid.  
5 to 10 grams of glycerine.  
45 2 liters of water.

The printing colours can be applied upon any ground color or the ground color can be obtained after printing.

After the printing operation has taken 50 place, the hides or skins are placed in a steam room, for about one hour, at a temperature of 75° C.

This steaming has for its purpose, the thor-

ough penetration of the dye-stuff which, prior to this operation, was but superficial. 55 Moreover this treatment in the steam room means a step towards the fixing which is effected by employing the usual pigments or mordants and is accomplished in a bath of emetic, such as tartar emetic, or of acid, according to the nature of the dye-stuffs used.

The acid or metallic mordants are employed to temporarily fix the dyestuffs which have been applied; but their main purpose is to form a chemical combination which intimately associates itself with the fibres of the leather, after a stay in the emetic and acid baths. Any color may be used in carrying out the process and as may be readily understood by those skilled in the art, the mordant employed will depend upon the color used. 65

The hides or skins are then washed in clear water; they are thus ready to be used for the manufacture of the articles for which they 75 are intended.

The leather thus printed retains, after washing all its properties as to softness and strength; moreover the penetration of the dye-stuff is deep enough, so that the colors 80 will not fade after a certain time of use.

It must be observed that the above figures and details for carrying out the invention have been given only by way of example and that they can be modified without departing 85 from the principle of the invention.

For instance, the tanning with formol could easily be replaced by a tawing process with the use of formol or alum.

What I claim is:

1. A process for the manufacture of washable printed leather which consists in preparing the hide or skin for the subsequent printing, steaming and fixing steps, by tanning the hide or skin first with formol, and 95 then tanning the same in a bath of powdered sumac.

2. In a production of washable color printed leather, the process which consists in subjecting the skin to successive tannings, first 100 with formol and then with sumac, and subsequently printing the same.

In testimony whereof I have signed this specification.

CHARLES S. FRIEDMAN.